# EUROPEAN PATENT APPLICATION

(11) **EP 0 318 231 A1**
(43) Date of publication of application: **31.05.1989**
(21) Application number: 88311004.1
(22) Date of filing: 21.11.1988
(51) Int. Cl.: C22B 34/12

(54) **Process for recovering titanium dioxide fines**

(30) Priority: 25.11.1987 US 125685
(71) Applicant: EXTRACT, INCORPORATED, Ashtabula Ohio 44004 (US)
(72) Inventor: Peterson, Richard B., Ohio 44004 (US); Muller, Kay Peterson, Ohio 44004 (US)
(74) Representative: Crisp, David Norman

(57) **Abstract**

A process for recovering titanium dioxide from a feed comprising titanium dioxide fines is disclosed. The process comprises the steps of (A) separating particulate matter having a Tyler Standard screen size of about 6 or larger from said feed; (B) removing liquid from said feed; (C) dividing said feed into (i) a concentrate having a relatively high concentration of titanium dioxide, (ii) middlings having a lower concentration of titanium dioxide than said concentrate, and (iii) tailings having a lower concentration of titanium dioxide than said middlings; and (D) removing liquid from said concentrate to form a product comprising titanium dioxide.

## Description

This invention relates to a process for recovering titanium dioxide and, more particularly, but not exclusively, to a process for recovering titanium dioxide fines that are in the form of particulate waste such as blow-over dust, cyclone solids and the like.

Titanium dioxide fines having a Tyler Standard screen mesh size of about 6 or finer, more often about 28 or finer, and in many instances about 200 or finer, are produced as by-products of various titanium compound production facilities such as, for example, titanium dioxide pigment plants and titanium tetrachloride plants. These fines are also produced as by-products in the mining of ilmenite and/or rutile. They are typically found in the waste streams of such titanium compound production facilities and mining operations and are usually disposed of in settling ponds and the like. These waste streams and settling ponds often contain other by-products such as coke, silica, and the chlorides and oxychlorides of various metals such as iron, vanadium, nickel, niobium, silver, tantalum, and the like. These fines have generally been regarded as waste products because it has not been economical to recover them in a usable manner.

J.I. Paige et al in "Physical Beneficiation of Titanium Plant Solid Wastes: Recovery of Titanium Minerals and Coke", Report of Investigations 8737, U.S. Department of the Interior, Bureau of Mines, report that they studied methods for recovering unreacted titanium minerals and petroleum coke from titanium chlorination plant wastes prior to neutralization treatment with lime. The objective was to recover valuable raw materials and to reduce the amount of waste materials that must be treated for disposal. Samples of solid wastes were physically beneficiated by gravity concentration (tabling) to recover titanium minerals containing 69.0 to 92.4% by weight TiO₂ and by selective carbon flotation to recover petroleum coke containing 94.0 to 96.8% by weight carbon. Laboratory data indicate that the recovered titanium mineral would decrease the amount of solid waste to be disposed of from 32.8 to 53.9% by weight. The recovery of coke would further decrease the amount by an additional 32.9% by weight. Tests conducted on recovering vanadium, chromium and columbium from liquors obtained by leaching chlorination residues indicated that (1) 97% of the vanadium was extracted from leach liquors in a two-stage solvent extraction procedure and (2) 58% of the columbium and 40% of the chromium were separated from the leach liquors by an ion exchange technique using a strong acid resin.

This invention provides for a process for recovering titanium dioxide from a feed comprising titanium dioxide fines, the process comprising:
(A) separating particulate matter having a Tyler Standard screen size of about 6 or larger from said feed;
(B) removing liquid from said feed;
(C) dividing said feed into (i) a concentrate having a relatively high concentration of titanium dioxide, (ii) middlings having a lower concentration of titanium dioxide than said concentrate, and (iii) tailings having a lower concentration of titanium dioxide than said middlings; and
(D) removing liquid from said concentrate to form a product comprising titanium dioxide.

Various preferred features and embodiments of the invention are described hereinafter.

The Figure of the accompanying drawing is a flow sheet schematically illustrating an embodiment of the invention by way of example.

The titanium dioxide fines that can be recovered in accordance with the inventive process typically have a Tyler Standard screen size of about 6 or finer, preferably about 28 or finer. Preferred particulate fines that can be recovered have a Tyler Standard screen size in the range of about 6 to about 600, more preferably about 28 to about 600. Advantageously, these fines have a Tyler Standard screen size in the range of about 6 to about 400, more preferably about 28 to about 400. These fines are sometimes referred to in the art as "blow-over dust" or "cyclone solids". Blow-over dust refers to the fact that the fines were entrained with a gaseous effluent of, for example, a fluidized bed reactor. Cyclone solids refers to the fact that the fines were collected in a cyclone.

These titanium dioxide fines are typically produced as by-products of titanium compound production processes (e.g., titanium dioxide pigment processes, titanium tetrachloride processes, and the like), rutile and ilmenite mining processes, and the like. These fines are usually found in the waste streams of such proces ses, and are typically disposed of in settling ponds, settling tanks and the like. The feed that is processed in accordance with inventive process is taken from these waste streams, settling ponds, settling tanks and the like. This feed typically contains, in addition to such titanium dioxide fines, other waste materials such as coke (or carbon), silica, and the chlorides and oxychlorides of various metals such as iron, vanadium, nickel, niobium, silver, tantalum and the like. The titanium dioxide fines can be in the form of titanium dioxide, rutile or ilmenite. The titanium dioxide fines can also be in the form of titanium-bearing compounds such as titanium-bearing ore and/or titanium-bearing slag. The coke can be in the form of petroleum coke and/or bituminous coke. The silica can be in the form of silica, quartz and/or calcined quartz. While the feed composition is dependent upon the particular process from which it is derived, it generally contains from about 20% to about 60% by weight solids, more typically from about 25% to about 50% by weight solids; and generally from about 40% to about 80% by weight liquid, more typically from about 50% to about 75% by weight liquid. The solids generally comprise from about 1% to about 50% by weight titanium dioxide, more typically from about 5% to about 40% by weight titanium dioxide; and generally from about 30% to about 99% coke, more typically from about 50% to about 95% by weight coke. The solids usually contain from about 10% to about 40% by weight titanium dioxide, from about 50% to about 80% by weight coke, and from about 10% to about 20% by weight silica. The liquid typically consists primarily of water, but can include acids such as hydrochloric acid and various dissolved metal chlorides and metal oxychlorides such as vanadium, nickel, niobium, silver, tantalum, and the like, at levels in the range of up to about 8% by weight.

The process will now be described with reference to the FIGURE. The feed is advanced to screen separator 10 to remove oversized particulate matter from the feed. Particulate solids having a Tyler Standard screen size of about 6 or larger, preferably about 28 or larger, are removed from the feed as oversized solids. Screen separator 10 is entirely conventional and can be, for example, a vibrating screen, a shaking screen, an oscillating screen, a reciprocating screen, a gyratory screen, etc. A Derrick Model J24-36-MS-1 vibrating screen adapted to separate out +28 Tyler Standard screen size solids is useful. Wash water can be added to the screen to enhance separation during screening. The ratio of wash water to feed that is added to screen 10 is dependent upon the nature and composition of the feed but can range up to, for example, about 6 gallons of water per dry net ton of feed. Feed and wash water passing through screen 10 are advanced to holding tank 12 where they are mixed with additional water plus filtrate recycled from filter 44 and overflow from cyclone 42, as discussed in greater detail below. The contents of tank 12 typically comprise about 12% to about 22% by weight solids, and about 78% to about 88% by weight liquid. The solids in tank 12 usually comprise from about 1% to about 50% by weight titanium dioxide and from about 30% to about 99% by weight coke. Oversized solids from screen 10 are collected for waste. The contents of tank 12 are advanced to cyclone 16 by pump 14.

Cyclone 16 is entirely conventional in design and preferably is adapted to separate out from the feed, as the cyclone overflow, liquids and particulate solids having a Tyler Standard screen size of about 600 or finer, generally about 400 or finer. The overflow from cyclone 16 typically has a solids content in the range of about 1% to about 15% by weight and a liquid content of from about 85% to about 99% by weight. The solids in the overflow typically have a titanium dioxide content of about 2% to about 10% by weight, and a coke content of about 30% to about 90% by weight. The underflow typically has a solids content of about 30% to about 70% by weight and a liquid content of from about 30% to about 70% by weight. The solids in the underflow typically have a titanium dioxide content of about 5% to about 70% by weight and a coke content of about 15% to about 65% by weight. Useful cyclones are available from Krebs Engineers under the names XZ Cyclones and Model D Cyclones.

The underflow from cyclone 16 is advanced to agitated tank 18 wherein it is agitated until it is advanced to stream splitter 22 by pump 20. Recycled middlings from concentrator tables 24, 26, 28, 30, 32 and 34, which are discussed below, are combined with the underflow from cyclone 16 prior to entering stream splitter 22. The combined underflow from cyclone 16 and recycled middlings generally have a solids content in the range of about 30% to about 60% by weight and a liquid content in the range of about 40% to about 70% by weight. The solids in the combined underflow and middlings generally have a titanium dioxide content of about 6% to about 70% by weight and a coke content of about 15% to about 65% by weight. Stream splitter 22 is adapt ed for dividing a slurry into a plurality of separate equal slurry streams. A useful stream splitter is available from the Deister Concentrator Company of Fort Wayne, Indiana under the name Deister Concenco Self-Propelled Splitter, Six-Way. In stream splitter 22, the combined underflow and middlings are divided into six separate feed streams.

The separate feed streams from streams splitter 22 are advanced to concentrator tables 24, 26, 28, 30, 32 and 34, respectively. The concentrator tables typically have a riffled plane surface inclined slightly from the horizontal. Separation between titanium dioxide and and the other solids in the feed is effected by flowing the feed across the plane surface which is differentially shaken in the direction of the long axis and washed with an even flow of water at right angles to the direction of motion. Separation depends mainly on the difference in specific gravity between the titanium dioxide and the other solids. Useful concentrator tables are available from Deister under the names DEISTER 999 Diagonal-Deck Ore Concentrating Table and SUPER DUTY Diagonal-Deck No. 6 and No. 14 Concentrating Tables.

The feed stream that is processed on each of the concentrator tables is divided into three separate product streams. The first of these separate product streams is a concentrate which has a relatively high concentration of titanium dioxide. Typically this concentrate has a solids content of about 30% to about 60% by weight and a liquid content of about 40% to about 70% by weight. The solids in the concentrate typically have a titanium dioxide content of about 90% to about 96% by weight, and a coke content of about 0.01% to about 1% by weight. The second of these separate streams is the middlings which has a lower concentration of titanium dioxide than the concentrate. Typically the midlings has a solids content in the range of about 50% to about 70% by weight and a liquid content in the range of about 30% to about 50% by weight. The solids in the middlings typically have a titanium dioxide content in the range of about 5% to about 70% by weight, and a coke content in the range of about 15% to about 55% by weight. The third is the tailings which has a lower concentration of titanium dioxide than the middlings. Typically the tailings has a solids content in the range of about 5% to about 27% by weight and a liquid content in the range of about 73% to about 95% by weight. The solids in the tailings typically have a titanium dioxide content in the range of about 1% to about 10% by weight, and a coke content in the range of about 20% to about 70% by weight. The concentrate streams from each of the concentrator tables are combined in tank 38. The middlings from each of the concentrator tables are combined, mixed with water, added to the feed stream from tank 18 and recycled to stream splitter 22. The tailings from each of the concentrator tables are combined and collected for waste.

The combined concentrate stream from tank 38 is advanced to cyclone 42 by pump 40. The overflow from cyclone 42 is recycled to either or both of tanks 12 and 38. Typically, from about 15% to about 40% by weight of the overflow is recycled to tank 12, and from about 60% to about 85% by weight is recycled to tank 38. The cyclone overflow consists primarily of liquid but can have a solids content of up to about 1% by weight. The underflow from cyclone 42 typically has a solids content of about 85% to about 90% by weight and a liquid content in the range of about 10% to about 15% by weight. The solids in the underflow typically has a titanium dioxide content in the range of about 90% to about 96% by weight, and a coke content in the range of about 0.01% to about 1% by weight.

The underflow from cyclone 42 is advanced to filter 44 wherein it is mixed with wash water and separated into a filtrate and a filter cake. Typically, from about 0.3 to about 5 gallons of wash water is added per gallon of slurry being treated in filter 44. Filter 44 is entirely conventional in design and can be, for example, a belt-vacuum filter. Particularly useful is the Eimco horizontal belt-vacuum filter which is available from Eimco Process Equipment Company, Salt Lake City, Utah.

The filter cake from filter 44 is advanced to bin 46 and from there to dryer 48 wherein remaining moisture is evaporated and a dried product is removed. The dried product preferably has a moisture content of about 3% by weight or less. Drying is preferably conducted at a temperature in the range of about 50°C to about 85°C. The dried product typically has a titanium dioxide content of at least about 90% by weight, generally from about 90% to about 96% by weight. The dried product can be stored in bins until it is ready for use, and can be advanced to such bins by conventional means such as conveyors or bucket elevators. The filtrate from filter 44 is advanced through trap 50 to tank 52, and then is recycled to tank 12 by pump 54.

The following example is illustrative of the process of the present invention. In the following example, as well as throughout the specification and in the appended claims, unless otherwise indicated, all parts and percentages are by weight, and all temperatures are in degrees centigrade.

### Example

The process depicted in the FIGURE, with changes as indicated below, was used. The flow rates and compositions of the initial feed, the final dried product and the various intermediate streams are indicated in the following Table. The screen 10 was a hand-held screen adapted for separating out particulate solids with a Tyler Standard screen size of 28 or larger. The cyclone 16 was a one-inch cyclone. Instead of using cyclone 42, liquid was decanted off the top. Only one concentrator table was used rather than the six concentrator tables 24, 26, 28, 30, 32 and 34 depicted in the FIGURE. The concentrator table that was used was a Deister single-deck ore concentrator table. The stream splitter 22 was not used. The filter 44 was a laboratory vacuum filter.

**TABLE**

| | Feed to Screen 10* | Feed to Cyclone 16 | Overflow to Cyclone 16 | Underflow to Cyclone 16 | Feed With Recycle to Splitter 22 | Overflow** Cyclone 42 | |
|---|---|---|---|---|---|---|---|
| Feed Rate (dry net tons/hr) | 4.50 | 4.50 | 0.32 | 4.19 | 4.81 | 0.01 | |
| TiO₂, % of solids | 25.50 | 25.50 | 4.74 | 27.06 | 27.06 | ---- | |
| Carbon, % of solids | 47.49 | 47.49 | 77.14 | 45.26 | 45.26 | ---- | |
| Solids, % | 30.00 | 16.46 | 1.55 | 60.00 | 39.86 | ---- | |
| Liquid, gal/hr | 2520.0 | 5480.0 | 4810.8 | 669.6 | 328.2 | 1099.2 | |
| Slurry flow rate, gal/hr | ---- | 6000.0 | 6000.0 | 1153.2 | 392.4 | ---- | |

| | Combined Streams From Tables 24-34*** | | | Underflow Cyclone 42 | Filter Cake Filter 44**** | Filtrate Filter 44 | Dried Product |
|---|---|---|---|---|---|---|---|
| | Concentrate | Middlings | Tailings | | | | |
| Feed Rate (dry net tons/hr) | 1.09 | 0.63 | 3.10 | 1.08 | 1.07 | 0.01 | 1.06 |
| TiO₂, % of solids | 93.80 | 27.06 | 3.59 | 93.80 | 93.80 | ---- | 93.80 |
| Carbon, % of solids | 0.12 | 45.26 | 61.13 | 0.12 | 0.12 | ---- | 0.12 |
| Solids, % | 50.00 | 60.00 | 20.92 | 65.00 | 88.0 | ---- | 100.0 |
| Liquid, gal/hr | 261.6 | 100.2 | 2808.0 | 139.2 | 32.4 | 227.4 | 0.0 |
| Slurry flow rate, gal/hr | 325.2 | 172.8 | 3228.0 | 204.0 | ---- | ---- | ---- |

| | | | | | | | |
|---|---|---|---|---|---|---|---|
| * Water added to screen at rate of 900.00 gal/hr. | | | | | | | |
| ** 121.8 gal/hr liquid + 0.01 dry net tons/hr solids recycled to tank 12. 977.4 gal/hr liquid recycled to tank 38. | | | | | | | |
| *** Water added to tables 24-34 at combined rate of 1200.0 gal/hr. | | | | | | | |
| **** Water added to filter 44 at rate of 120.0 gal/hr. | | | | | | | |

While the invention has been explained in relation to its preferred embodiments, it is to be understood that various modifications thereof will become apparent to those skilled in the art upon reading the specification.

## Claims

1. A process for recovering titanium dioxide from a feed comprising titanium dioxide fines, the process comprising:
(A) separating particulate matter having a Tyler Standard screen size of about 6 or larger from said feed;
(B) removing liquid from said feed;
(C) dividing said feed into (i) a concentrate having a relatively high concentration of titanium dioxide, (ii) middlings having a lower concentration of titanium dioxide than said concentrate, and (iii) tailings having a lower concentration of titanium dioxide than said middlings; and
(D) removing liquid from said concentrate to form a product comprising titanium dioxide.

2. The process of claim 1 with the step of combining said middlings from step (C) with said feed from step (B).

3. The process of either of claims 1 and 2 with the step of dividing said feed from step (B) into a plurality of separate feed streams prior to step (C), dividing each of said separate feed streams during step (C) into separate concentrate streams, middlings streams and tailings streams, and combining said separate concentrate streams to form said concentrate prior to step (D).

4. The process of claim 3 with the steps of combining said separate middlings streams to form a combined middlings stream, and combining said combined middlings stream with said feed from step (B) prior to step (C).

5. The process of any preceding claim wherein said feed is tabled during step (C).

6. The process of any preceding claim wherein step (D) includes the step of filtering said concentrate to form a filtrate and a filter cake, said filtrate being combined with said feed from step (A) prior to step (B).

7. The process of claim 6 with the step of drying said filter cake to form a dried product comprising titanium dioxide.

8. The process of any preceding claim wherein said feed comprises blow-over dust.

9. The process of any preceding claim wherein said feed comprises titanium dioxide and coke prior to step (A).

10. The process of any preceding claim wherein said product from step (D) has a moisture content of about 3% by weight or less.
